

# UNITED STATES PATENT OFFICE.

JEAN BILLITER, OF VIENNA, AUSTRIA-HUNGARY.

## SELF-IGNITING ELECTRIC-ARC CANDLE.

1,216,404.

Specification of Letters Patent. Patented Feb. 20, 1917.

No Drawing.

Application filed January 28, 1914. Serial No. 815,065.

*To all whom it may concern:*

Be it known that I, JEAN BILLITER, a subject of the Emperor of Austria-Hungary, residing at 16 Pelikangasse, Vienna, in Austria-Hungary, have invented certain new and useful Improvements in Self-Igniting Electric-Arc Candles, of which the following is a specification.

It is a well known fact that the ignition of electric arc lamp candles consisting of two parallel electrodes and an intermediate layer between said electrodes offers such difficulties that notwithstanding their simplicity they have hitherto not found a general introduction. A great number of contrivances have been devised with the object of mechanically effecting the ignition, for instance by approaching the electrodes to each other and again separating them, by introducing an intermediate member, and the like. But with all such arrangements the essential feature of these candles (simplicity) is lost, and the intricate mechanism renders the lamp complicated, affects the arc, consumes energy, and the like.

The experiments which have heretofore been made to obtain a re-ignition of the electric arc, after it has been extinguished, by means of chemical changes in the intermediate layer, have not been successful. For instance, it has been proposed (German Patent No. 8785) to fill the intermediate layer between the electrodes with semi-conductors such as anthracite or a mixture of a powdered metal, say 0-10% zinc with non-conductive substances as magnesia, magnesia cement or a mixture of metal oxids, which are reduced to their respective metal in the electric arc, with magnesia cement and the like. Under the action of the electric arc a conductive layer is actually formed which will bridge the gap between the electrodes (hereinafter such layer will be briefly termed the "bridge") and which may effect an ignition of the electric arc when the current is switched on. However, secondary effects will appear, which entirely destroy the advantages obtained.

The arc, for instance, quickly fuses the material of the intermediate layer or bridges will be formed in the deeper strata of the intermediate layer, so that its electrolytic or metallic conductivity is so far increased that the electric current will tend to pass through the intermediate layer only.

The applicant has already proposed a universal means for obtaining conductive bridges of a small sectional area only, which will not increase in size as hereinbefore described by choosing as components of the bridge forming layer, igniting substances or mixtures of substances which pass at higher temperatures *i. e.* for example above 200°, from the non-conducting or badly conducting state through a chemical process 60 into a good conducting state by forming conducting compounds, as carbids, lower oxids or corresponding compounds.

For making the intermediate layer therefore there is used preferably a mixture of a carrying substance, the composition of which is immaterial for the purpose of the present invention, as magnesia and silicic acid, or water glass (sodium or potassium silicate), fire brick and silicic acid or even oxalate or carbonate in connection with a flux and a binding substance; and to this mixture are added, in order to form the bridge, substances, which when heated form conductive compounds, as lower oxids or carbids by a 70 chemical process. Preferably I propose compounds of multivalent metals as titanium, cerium, thorium, zirconium, etc., for instance titanium salt, or titanium oxid (rutile), titanic acid or the like or mixtures 75 of metal oxids, for instance a mixture of thorium oxid and lanthanum oxid.

To enable any one skilled in the art to make a candle which will relight in the aforesaid manner I will give hereafter the 80 proportion of the substances used to make the bridge forming layer of a candle.

I use:

|                                                                                                                       |            |
|-----------------------------------------------------------------------------------------------------------------------|------------|
| (1) Carrying substances (magnesia oxid, fluorspar, cryolite or the like) -----                                        | 95         |
| (2) Bridge-forming substances (titanium oxid, vanadium oxalate, cerium oxid or the like) -----                        | 20-80% 100 |
| (3) Flux (boric acid) -----                                                                                           | 0-5%       |
| (4) Binding medium (adhesive solution of titanium oxalate or titanium formate or molybodic oxalate or the like) ----- | 25-50% 105 |
| (5) Addition (graphite) -----                                                                                         | 2-20% 110  |

Within these limits the proportions must be chosen according to manner of the electric current (direct or alternate current) and according to the intensity of the current.

When using direct current and candles employed with an intensity of current of 8-12 amperes the best proportions are:

5 Fluorspar as carrying substance 100 g.  
Titanium acid anhydrid as bridge forming substance 100 g.  
Boric acid as a flux 8 g.  
Binding substance 100 g.  
10 Graphite as addition 30 g.

These combinations pass over to the conducting condition only at relatively high temperatures, so that the desired effect of keeping the bridge is thus attained. A further advantage consists in the fact that these conducting bridges remain conducting also after being cooled, whereas the substances formerly proposed can easily pass into the non-conducting state of oxidation.

15 20 For producing the first ignition the bridging substance above or the points of the electrodes in addition are covered with a thin layer containing a finely distributed metallic conducting powder, in which the arc produced when the current is switched on will immediately form a bridge.

I claim:

1. A self-igniting arc lamp candle comprising juxtaposed electrodes and an intermediate layer between said electrodes consisting of 20-60% titanium oxalate or its described equivalents being the bridge-forming substance, 20-80% fluorspar or the described equivalents being the carrying substance, 25-50% solution preferably adhesive 35 solution of titanium oxalate or the described equivalents being the binding substance and 2-20% graphite or the described equivalents.

2. The herein described composition of matter for forming the intermediate layer 40 of a self-igniting electric arc light candle consisting of fluorspar 100 g., titanium acid anhydrid 100 g., boric acid 8 g., binding substance 100 g., graphite 30 g. substantially as described.

In testimony whereof I affix my signature in presence of two witnesses.

DR. JEAN BILLITER.

Witnesses:

AUGUST FUGGER,  
ADA MARIA BERGER.

Copies of this patent may be obtained for five cents each, by addressing the "Commissioner of Patents, Washington, D. C."